

# UNITED STATES PATENT OFFICE.

CARLETON ELLIS, OF MONTCLAIR, NEW JERSEY, ASSIGNOR TO ELLIS-FOSTER CO., A CORPORATION OF NEW JERSEY.

## DESULFURIZING CAST-IRON.

1,335,370.

Specification of Letters Patent. Patented Mar. 30, 1920.

No Drawing.

Application filed October 9, 1917. Serial No. 185,552.

*To all whom it may concern:*

Be it known that I, CARLETON ELLIS, a citizen of the United States, and a resident of Montclair, in the county of Essex and State of New Jersey, have invented certain new and useful Improvements in Desulfurizing Cast-Iron, of which the following is a specification.

This invention relates to a process of desulfurizing cast iron and the like and has to do particularly with the treatment of sulfur-bearing cast iron, with calcium or similar element, in the form of a compound with certain other elements which enable the full reactive qualities of the element calcium to be exerted in desulfurization. The method also may be employed in the case of iron containing phosphorus and silicon in excessive quantities.

A good part of the iron cast in foundries is made by melting scrap. Sometimes ordinary pig iron is added but often a large part of or the entire charge in the cupola is scrap iron stock. This is melted by means of coke containing sulfur, and a certain amount of sulfur thus is imparted to the cast iron each time a charge is run. Consequently each time scrap iron is remelted, sulfur is introduced and therefore it follows that the entire supply of pig iron is increasing in average sulfur content through such repeated melting. Furthermore the coke available at many points is, if anything, tending gradually to run higher in sulfur, which aggravates the condition. After iron has been charged with a certain amount of sulfur it becomes hot short and has other objectionable qualities. Usually a proportion of sulfur of above one per cent. renders the iron unworkable for many purposes. For example, .9% of sulfur is the maximum amount of sulfur permitted in certain cases.

It is possible to blow air through the molten iron in a converter, especially one equipped with a basic lining to oxidize and remove the sulfur and produce a species of steel or pure iron which may be incorporated with some of the original iron so that the resulting melt contains less than 1% of sulfur, or whatever the maximum sulfur content may be permitted under the circumstances. By such blowing operation the content of carbon is usually reduced, sometimes to an undesirable point and powdered coal or coke or other form of carbon may

be added to the iron until its content of carbon is brought up to the requisite point. Or the blown iron practically free from sulfur and silica may be recarburized by treatment with coal or coke.

Such a procedure however, involves complicated and expensive equipment and careful operation and control such as often is not feasible in ordinary foundry practice and in the present invention the object is more particularly to provide a means for treating sulfur containing iron in the ladle or other container into which the molten iron is run, for example, from the cupola or in some other simple way contacting the sulfur-containing iron with the desulfurizing reagent so as to enable the process to be used in ordinary foundry operations without complicated apparatus.

The particular form of desulfurizing agent which I prefer to use in the present invention is a calcium compound containing the element calcium in such a state as to readily combine with sulfur, phosphorus, silicon, and the like and having no other element in combination with the calcium which would be objectionable in the iron. For example I may use calcium cyanamid as a desulfurizing agent and when this comes in contact with molten cast iron and reacts with the sulfur therein the carbon and nitrogen of the cyanamid are not objectionable constituents under these conditions. If on the other hand, molten iron is treated with calcium oxid the effect is rather to produce a slag with silicious material than to bring about an effective combination with sulfur. Metallic calcium would be an excellent desulfurizing agent from the standpoint of efficiency but is too expensive. Oxids of calcium are far less active because the affinity of the calcium is already satisfied to a large extent by the oxygen with which it is combined. In the case of calcium cyanamid, however, the combination is not a highly stable one and the calcium is much more free to combine with the sulfur especially in view of the affinity of iron for carbon. By the use of material such as calcium carbid or calcium cyanamid the effect of metallic calcium is obtained in a way without resorting to anything as expensive and as difficult to preserve as calcium in the metallic state.

The reagent may be mixed in lump or

powdered form with the iron in the form of 5 turnings, shavings and the like, and may be melted to bring about the reaction or the product may be placed in the bottom of the ladle and the molten iron from the cupola or other container run therein, when reaction takes place. Or the ladle may be lined with a mixture comprising calcium carbid, calcium cyanamid or similar calcium compound. 10 Or the iron may be allowed to flow along a trough lined with material containing the carbid, nitrid or the like.

In one case the treatment of cast iron with calcium carbid, the original content of the 15 iron being 0.93% sulfur and 2.42% silicon, the sulfur was reduced to 0.65% and the silicon to 1.98%. Similarly with calcium cyanamid a reduction in sulfur and silicon content occurred, the degree of reduction in the 20 case of the silicon being greater than with the calcium carbid employed under the conditions of the test.

Thus it will be seen that the essence of the invention consists in treating under suitable 25 reacting conditions cast iron containing sulfur, phosphorus, silicon and the like, (one or more of these impurifying elements being present, as the case may be) with a reagent, namely, a compound containing an element 30 of a basic character such as the alkaline earth metals, namely: magnesium, calcium, barium, etc., or even the alkali metals such as sodium in combination with an element or radical which yields a compound capable 35 of being readily handled but which does not impair to any objectionable extent the reactivity of the basic element in question. For example, the elements calcium, barium, sodium and the like, may be combined with 40 carbon to form a carbid; with nitrogen, to make a nitrid; with hydrogen, to yield a hydrid; with carbon and nitrogen, in the case of calcium, for instance, to give the cyanamid. Preferably the element of calcium 45 or other alkali material is combined

with a non-metallic element or metalloid or grouping of metalloidal elements. Hence the carbid or nitrid, for example, has a preference over a body of the nature of the hydrid.

Manganese may form a part of the desulfurizing agent under some circumstances such as additions of manganese in the form of ferro-manganese and the like may be employed along with the calcium cyanamid or 55 similar desulfurizing agent.

What I claim is:—

1. The process of desulfurizing cast iron which comprises bringing calcium cyanamid into contact with the molten metal.

2. The process of desulfurizing cast iron which comprises running molten cast iron containing sulfur into a ladle containing calcium cyanamid.

3. The process of desulfurizing cast iron 65 which comprises bringing a basic cyanamid into contact with the molten metal; the base of said cyanamid being capable of uniting with some portion at least of the sulfur in the cast iron and separating from the latter 70 as slag.

4. The process of desulfurizing cast iron which comprises running molten cast iron 75 containing sulfur into a ladle containing a basic cyanamid, the base of said cyanamid being capable of uniting with some portion at least of the sulfur in the cast iron and separating from the latter as slag.

5. The process of desulfurizing cast iron which comprises bringing molten cast iron 80 containing sulfur into contact with a mixture comprising calcium cyanamid and calcium carbid.

6. The process of desulfurizing cast iron which comprises bringing into contact with 85 the molten metal a desulfurizing agent comprising calcium united with an element whose liberation in the iron does not materially affect the quality thereof.

CARLETON ELLIS.